

# UNITED STATES PATENT OFFICE.

CONSTANTIN JEAN TOSSIZZA, OF PARIS, FRANCE.

## ELECTROMETALLURGIC TREATMENT OF ORES OF COPPER OR OTHER METALS.

SPECIFICATION forming part of Letters Patent No. 710,346, dated September 30, 1902.

Application filed August 6, 1901. Serial No. 71,104. (No specimens.)

*To all whom it may concern:*

Be it known that I, CONSTANTIN JEAN TOS-  
SIZZA, a citizen of the Republic of France, re-  
siding at Paris, France, have invented a new  
5 and useful Improvement in Electrometallur-  
gic Treatment of Ores of Copper, &c., of which  
the following is a specification.

The direct electrolytic treatment with in-  
soluble anodes of the solutions obtained by the  
10 action of sulfuric acid on previously-roasted  
copper ores has heretofore been impractical-  
able, because it required, before all, a complete  
purification of the solutions obtained in or-  
der to free them of all sulfates other than the  
15 sulfate of copper. Such a purification being  
very difficult, the direct electrolytic treat-  
ment was for that reason industrially inap-  
plicable.

The present invention has for its object to  
20 make possible the said electrolytic treatment  
without preliminary purification.

A solution of the sulfates from treating  
copper ores contains besides the sulfate of  
25 copper the sulfates of other metals and in  
particular the sulfate of iron. Among all  
these sulfates that which is decomposed at  
the lowest voltage is sulfate of copper. The-  
oretically, then, by effecting the electrolysis at  
30 a voltage sufficiently high to decompose the  
sulfate of copper and not high enough to de-  
compose the sulfates of iron and other met-  
als a pure electrolytic deposit of copper ought  
to be obtained; but in working with insolu-  
35 ble anodes incidental phenomena of polariza-  
tion do not permit the practical realization  
of the indispensable theoretic condition—  
to wit, the maintenance of a constant voltage  
between very restricted limits. The poten-  
40 tial at the poles of the electrolytic cell is not  
slow to rise, and the metallic deposit, which  
in the first instants of the operation was  
formed of pure copper, quickly becomes im-  
pure and formed almost exclusively of spongy  
45 iron. It is necessary, then, in order that the  
operation may be possible to be able to keep  
uniform the voltage first established. This  
result could be obtained by the use of soluble  
metallic anodes; but in working to avoid the  
50 electrolysis of the iron it would be necessary  
for the said electrodes to be such as by their

solution to yield an electromotive force less  
than that for the decomposition of iron. It  
would be necessary, then, to use copper elec-  
trodes, which would render the system im-  
practicable, because there would be dissolved 55  
at the anode exactly the quantity of cop-  
per deposited at the cathode. Under these  
conditions I have thought to use in place of  
soluble electrodes insoluble anodes kept in  
60 contact with sulfuric acid, and thus to util-  
ize the known depolarization properties of  
the said sulfuric acid. These anodes can  
be made of carbon, and in this case the sul-  
furic acid can be introduced outside the 65  
anode or in the interior thereof, if the anode  
is hollow, and it may be in the state of a so-  
lution or in the gaseous state.

I have ascertained that the transforma-  
tion of the sulfuric acid into sulfuric acid  
at the anode gives rise to an electromotive 70  
force which diminishes the necessary voltage  
and lowers it to two-tenths of a volt. One  
can thus obtain a very beautiful deposit of  
pure electrolytic copper directly from an im-  
pure solution with a sufficient intensity at a 75  
voltage of about six-tenths of a volt, whereas  
in all processes heretofore known one could  
only obtain this electrolysis with insoluble  
anodes at voltages above one and three-tenths  
volts. Incidentally I may remark that the 80  
copper thus obtained being tenacious and  
ductile is directly laminable or it can be de-  
posited directly in the form of tubes which  
can be employed in industry.

It results from the preceding that sulfur-  
ous acid, which has been considered an ob-  
jectionable element in metallurgy and which  
it has been sought to get rid of as much as  
possible, becomes an auxiliary in electromet-  
allurgy and makes it possible to manufacture 90  
metals at voltages inferior to those of their  
theoretical formation in their direct or indi-  
rect electrolysis.

The sulfuric acid introduced into the elec-  
trolytic bath is preferably obtained from the 95  
preliminary treatment of the ores. Copper  
and most metals exist in the form of sulfid  
ores, which when roasted produce oxids and  
sulfurous acid. The oxids are transformed  
into sulfids by dissolving them in sulfuric 100

acid. The sulfurous acid is dissolved in water and the solution introduced into the electrolytic bath.

I claim—

- 5 1. The process of treating electrolytically the impure and ferruginous solutions of sulfate of copper obtainable by the solution of copper ores in sulfuric acid, in order to recover the copper electrolytically without special preparation, by proceeding with the electrolytic treatment at a voltage between about two-tenths and eight-tenths of a volt with insoluble anodes maintained in contact with sulfurous acid, substantially as described.
- 15 2. In the electrolytic decomposition of the impure solutions obtained by roasting sulfid ores and dissolving the products of such roasting, the process of recovering a metal from

said solution without preliminary treatment to remove another metal or other metals present therein, consisting in introducing sulfurous acid from the said roasting operation into the electrolytic bath, while at the same time adjusting the voltage in such manner as to effect the decomposition of the salts of the metal to be recovered and not of the other metals present in said solution, substantially as described.

In witness whereof I have hereunto signed my name in the presence of two subscribing witnesses.

CONSTANTIN JEAN TOSSIZZA.

Witnesses:

JULES ARMENGAUD, Jr.,  
MARCEL ARMENGAUD, Jr.